

May 18, 1926.

1,584,959

C. P. MADSEN

ELECTRODEPOSITED METAL

Original Filed April 26, 1919

FIG. 1.



FIG. 2.

Inventor

Charles P. Madsen

Witness  
Floyd A. Cornwall  
Philip E. Everett  
By Emery Varney, Blair & Hogan  
his attorneys

Patented May 18, 1926.

## UNITED STATES PATENT OFFICE.

CHARLES P. MADSEN, OF NEWARK, NEW JERSEY, ASSIGNOR TO MADSENELL CORPORATION, OF NEW YORK, N. Y., A CORPORATION OF NEW YORK.

## ELECTRODEPOSITED METAL.

Application filed April 26, 1919, Serial No. 292,794. Renewed July 28, 1925.

The present invention relates to electrodeposited metals, particularly what I term the "nickel metals", such as nickel, or cobalt, or metal alloys containing substantial percentages of either nickel or of cobalt, or both nickel and cobalt. It is the object of the present invention to provide such "nickel metals" in a condition in which the same will possess new and extremely valuable properties enabling such "nickel metals" to be put to a wide variety of important uses for which nickel, or cobalt or alloys of either or both of these metals, as prepared by the customary metallurgical or electrodeposition methods, have hitherto been unavailable.

The present application is a continuation in part of my copending applications Ser. No. 254,793, filed September 19, 1918, and Ser. No. 317,656, filed August 15, 1919.

By way of example, I shall describe herein in detail an illustrative embodiment of my invention particularly as applied to produce electrodeposited nickel in a dense, reguline condition, which metal is substantially free from pits, pores and hydrogen, and is at the same time malleable and ductile to a remarkable degree. For example, the nickel product comprising said illustrative embodiment is more workable than hard-rolled copper, even more workable than brass, and almost as workable as soft-rolled copper.

It should however be clearly understood that cobalt or alloys containing substantial percentages of either nickel or cobalt or of both these metals, may be produced by means analogous to those herein described for the production of my new kind of nickel and possessing the advantageous properties referred to in connection with said new kind of nickel.

In producing the foregoing new nickel of my invention, comprising one illustrative embodiment of said invention, I may use an electrodeposition bath of the following composition: Nickel sulphate 240 g., nickel chloride 20 g., boric acid 40 g., water 1 liter.

This bath is preferably operated at a temperature of about 130° F. Except for the addition of boric acid, as set forth above, the bath should be neutral. The anode may consist of cast or rolled nickel, and the cathode of a metal, such as aluminum or nickel, which is adapted to receive

a smooth, separable deposit of the electrodeposited nickel. However, if so desired, the metal may be electrodeposited adherently, as in the form of a plating, which will adhere closely to the cathode if the latter is not given any special treatment to render the deposit readily removable and non-adherent.

During deposition the cathode on which the nickel is being electrodeposited, is intermittently or periodically exposed to a gaseous medium, such as the air, as by removal from the bath or otherwise. The time during which the cathode and the electrodeposited nickel carried by it are kept out of the bath should be more than what I term the "minimum" or "hydrogen dissipation" period, which is necessary to permit the hydrogen deposited with the metal to be dissipated or removed by contact with the surrounding gaseous medium, such as the air. This "minimum" or "hydrogen dissipation" period may be readily determined by trial and experiment and is generally greater than about one second, usually two seconds.

The time during which the cathode and the deposit carried by it are kept out of the bath should not, however, exceed what I term the "maximum" or "critical" or "separable deposit" period, which, in the case here given, is from about 6 to about 16 seconds, by which I mean that if the time during which the cathode and its deposit are kept out of the bath exceeds the said "maximum" or "critical" or "separable deposit" period, on restoring the cathode and its deposit to the bath, the succeeding deposit will not be adherent but will separate or be easily separable from the previous deposit. This results in a laminated, weak metal, a condition which is obviously to be avoided, where a sound unitary metal is desired.

The frequency of removal or "exposure frequency period" is determined by the factors of deposition which influence hydrogen liberation, such as the degree of exactness of neutrality, current density, and temperature. I have found that in the bath here described by way of example, and operating at a temperature of about 130° F., and with a current density of about 10 amperes per square decimeter, this period may be from 1 to 2 minutes.

In order, moreover, that the electrodeposited metal, such as the nickel in the example

given, may not only be dense, reguline and free from pores and hydrogen, but in order also that said metal shall be free from what are known as "pits" in the art of the deposition of the "nickel metals," I add to the bath, preferably before starting the electrodeposition, a quantity of finely divided nickel hydrate, preferably freshly precipitated nickel hydrate ( $\text{NiO}_2\text{H}_2$ ) and probably existing in a colloidal condition, which nickel hydrate remains in suspension in the bath during electrodeposition. While the quantity of hydrate so added may vary within considerable limits, I prefer to add from 1 to 5 grams, generally 1 gram, of said colloidal nickel hydrate to each liter of bath solution.

I have discovered that by adding to the bath certain salts, such as the sulphates, of the alkali metals, preferably sodium, finely divided or colloidal nickel hydrate is produced and held in suspension in the bath. This freshly and continuously produced hydrate replenishes the hydrate which during the operation of the bath aggregates or for other reasons goes out of suspension and drops to the bottom of the bath. Such salts have further beneficial effects and greatly improve the operation of the bath and the character of the deposits formed. For this purpose I may add varying amounts, such as from about 1 to about 10 grams, preferably 1 gram, of sodium sulphate for each liter of bath solution.

The action of the colloid-producing substance, such as the sodium sulphate, described above, is to produce by and during electrodeposition, some caustic soda or sodium hydroxide. The caustic soda or sodium hydroxide thus produced, by interaction with the nickel salts present in the bath, such as the nickel sulphate, generates finely divided or colloidal nickel hydrate which remains suspended in the bath. The interaction at the same time re-generates the sodium sulphate. The sodium sulphate or its equivalent also acts to assist the deposition and to improve the character of the deposit, which factors are also further assisted by the initial addition of nickel hydrate in finely divided or colloidal condition to the bath.

In the accompanying drawing, I have diagrammatically illustrated a form of apparatus in which the foregoing illustrative embodiment of my invention may be carried out.

Referring to these drawings:

Figure 1 is a cross section; and

Figure 2 is a longitudinal section of such apparatus.

The apparatus comprises briefly, a vat 1, for containing the bath 2. 3 is the anode and 4 the connector for supplying said anode with current. The cathode is indicated at 5 and its conductor at 6. At 7 is indicated

generally any suitable means, which may, if desired be manually operated, for intermittently or periodically removing the cathode from the bath, as set forth above.

The resulting product, as in the case of nickel in the illustrative embodiment set forth above, is, as before stated, dense, reguline, homogeneous, malleable and ductile. The new nickel herein described is substantially free from pores and pits and contains no appreciable amount of hydrogen.

It is of course, to be understood that where a deposit of cobalt, having the foregoing desirable properties, is desired to be produced, a cobalt anode is used in place of the nickel anode, and cobalt compounds are used in place of the corresponding nickel compounds. Where alloys of either nickel or of cobalt or of both of these metals are desired to be produced, means analogous to the means herein set forth for the deposition of nickel and of cobalt in the desired condition and having the desired properties may be employed.

The nickel herein described differs in character from the nickel obtained by the usual metallurgical processes in that my new nickel is free from the usual "poisonous" contents such as sulphur, silicon, arsenic, carbon, carbides, oxygen, and other gases and oxide containing compounds, generally present in metallurgical nickel and rendering the same imperfect and more difficult to work.

Furthermore, my new nickel is to be further differentiated from the ordinary metallurgical nickel in that it has a finer and more even grain than such metallurgical nickel, as is shown by metallographic micro-photographs. It is also considerably purer than such metallurgical nickel, resists chemical action better and has a higher melting point.

The nickel described herein is also to be differentiated from the usual electrodeposited nickel in that it is substantially free from pores, pits and hydrogen, and is malleable and ductile to a very high degree, unlike the usual electrodeposited nickel which is porous, contains a large hydrogen content and is brittle and unworkable.

A further difference in character between my new nickel and the ordinary metallurgical nickel is shown by the fact that the film of oxide formed by heating my new nickel in an oxidizing atmosphere is thinner, finer in texture and more adherent and flexible than the oxide coating formed by similar treatment of ordinary metallurgical nickel. Furthermore, such oxide coating in the case of my new nickel is of a different color, generally yellow to brown, while the oxide coating on the metallurgical nickel is generally violet or indigo in color.

It is of course, to be understood that the invention is not to be limited to the specific illustrative embodiment herein described for

purposes of example only. It is also to be understood that the applicant does not wish to have the invention or the appended claims in any way limited by and particular theory 5 of operation which he may now hold and which may be suggested by the foregoing detailed description.

What I claim is:

1. As an article of manufacture, electro-  
10 deposited "nickel metal" of a dense, regu-  
line structure, being malleable and ductile,

and substantially free from pores, pits and hydrogen.

2. As an article of manufacture, substan-  
tially pure electrodeposited nickel of a dense, 15  
reguline structure, being malleable and duc-  
tile, and substantially free from pores, pits  
and hydrogen.

In testimony whereof, I have signed my  
name to this specification this 26th day of 20  
April 1919.

CHARLES P. MADSEN.